

## UNITED STATES PATENT OFFICE

2,685,438

PROCESS FOR THE SOLUTION MINING OF  
POTASSIUM COMPOUNDSWalter M. Cross, Jr., Kansas City, Mo., assignor  
to Kansas City Testing Laboratory, Kansas  
City, Mo., a corporation of MissouriNo Drawing. Application June 30, 1948,  
Serial No. 36,271

3 Claims. (Cl. 262—3)

1

This invention relates to an improved process of recovering potassium salts from brines and ores. More particularly, this process pertains to a method of eliminating the interference of certain salts which may periodically be present in solution mining when an ore variant in potassium concentration is mined.

Present methods of mining potash are akin to shaft, room and pillar type of mining, or of the solution type, several of which methods are described in Patents No. 2,161,800 issued June 13, 1939, and No. 2,331,890, issued October 19, 1943, granted to Dr. Roy Cross and assigned to the assignee of the present application.

In solution mining of potash superheated liquor may be introduced to a potash bed or beds, thereby dissolving a mixture of salts containing potash. The salt solution is subsequently cooled, whereby potash is deposited out from the saturated salt liquor. In another method of solution mining substantially all of the potash salts are removed from salt deposits of potassium chloride and sodium chloride, leaving most of the sodium chloride in situ when a superheated mother liquor is used which is a solution substantially saturated with respect to both sodium chloride and potassium chloride. This method proceeds on the theory that solubility of potash salts is proportional to increase of the temperature of the dissolving medium. The solubility of the potash salts is greater than some other salts; sodium salts for example. When a superheated solution is introduced greater quantities of potash are dissolved and less amounts of other salts. Solutions of higher potash concentration are obtained by solutions which will take up only potash salts. Accordingly, hot solutions which are already saturated with undesirable salts are employed circulated into potash deposits. An equilibrium of solution between potash salts and other salts occurs, and the solution takes up potash salts since it is already saturated as to the undesirable salts found in the deposit.

A problem encountered in either of the above described solution mining methods has occurred where the potash beds so mined contain either magnesium or sulphate compounds or both. Salts of this type serve to saturate the dissolving mother liquor to the exclusion of the potash salts. It therefore becomes necessary when these salts are encountered in the mining operation to raise the saturation ability of potash in the brine or other solution introduced so as to dissolve the salt bed so that less water is required to be evaporated in the recovery of each potash unit.

Evaporation is an expensive operation and a means for reducing the proportions of such operation decreases commensurately with the cost of over-all mining operation. Hence, the expense involved for mining a unit of potash, be it pound, barrel or ton, is also decreased.

I have discovered that the depressant effect of magnesium and sulphate salts may be removed by changing such salts to a hydroxyl form. Such change serves to render magnesium or sulphate ions either relatively insoluble or inactive as to the inhibition of the solubility of potassium.

The novelty in the method herewith described is that in above ground operations upon crushed ore, the ore in leaching operations is under control, and the potash content of the ore is of sufficient concentration to permit excellent potash saturation. But in operating under ground, it is impossible to choose the type of ore for operation, and in the case where the ore is not rich, the law of mass reaction becomes operative. This is of great consternation. Thus, as an example, where sodium chloride is present in the ore beds, it goes into solution in the mother liquor introduced in preference to the potash salts. Variant temperature control of the mother liquor only indicates that at a higher temperature, more salt is taken up. Though in a pure water solution the solubility of potassium chloride is greater than that of sodium chloride, in a solution of water with a mixture of the two salts the rate of solution of sodium chloride is faster. It becomes necessary, therefore, to eliminate as many factors which tend to depress the solubility of the potash salts, so as to maintain an operable potassium chloride-sodium chloride ratio.

In a typical well in a potash bed the following may be descriptive of my operation: Normally, a value of 1½ pounds potassium chloride to one gallon brine is obtained. In a typical instance this value may fall to 0.3 lb./gal. At this point the particular ore reaches an equilibrium. The underground pool is estimated at 150 barrels volume. In order to raise the saturation of potash in the brine, I treat the brine with sodium hydroxide in order to convert magnesium chloride, for example, to magnesium hydroxide. This raises the potassium chloride concentration, and in one instance, specifically raised the value of concentration of potassium chloride from 0.3 lb./gal. to 0.5 lb./gal. In point of time this saturation increase is immediate; in typical operation an increase of saturation of 0.2 lb./gal. is obtained in one hour. In other instances a saturation figure of less than 0.3 lb./gal. has been

raised to 0.6 lb./gal. Higher concentration is important since less evaporation is required to recover potash with consequent decrease in operating costs.

Treatment with calcium hydroxide yields equally good results. Both agents serve chiefly to convert magnesium chloride into magnesium hydroxide, a compound of relative insolubility.

Where calcium sulphate is present it is converted to calcium hydroxide. Reagents which are suitable for such conversion may be caustic soda or lime, the latter being more suitable because of its cheapness. In a mixture of salts comprising potash and salts containing the hydroxyl ion, the hydroxyl ion is of little depressant effect, whereas the soluble magnesium and sulphate ions serve to cause difficulty by readily going into solution and by displacing the desirable potassium ions. Calcium sulphate may be eliminated by using soda ash or a chemical of the tri-sodium phosphate type.

This method makes solution mining possible without superheating the mother liquor used to dissolve the potash beds. Cold water will serve to yield the results as above described.

The conversion of undesirable ions into a non-interfering form is operative when the alkaline reagent is in sufficient quantity to keep the dissolving brine at a pH of 8.0 to 10.0. Treating the mother liquor so as to impart this pH may be done in advance of actual operations or concurrent with the pumping operation or after the mining cycle is in operation. Since there is no critical phase in the operation when the alkalinity must be imparted, the process herein described may be undertaken in all solution mining processes heretofore or currently employed. There is no limitation upon use of the alkaline material with respect to temperature. Therefore, the solutions used in my mining methods described in my patents already issued may be treated to a point of alkalinity so as to avoid the interference of the kind described herein. An optimum range of operation for effecting the benefits of this method may be obtained by bringing the mother liquor to a pH of 8 to 10.

What I claim is as follows:

1. A cyclic process for the solution mining of potassium compounds from underground water soluble deposits containing potassium, magnesium and sulfate ions which comprises circulating a body of aqueous solvent liquor unsaturated with respect to potassium compounds into contact with said deposits, adding a quantity of sodium hydroxide sufficient to raise the pH of

said liquor to between 8 and 10 thereby to repress the solubility of the magnesium and sulfate ions in said liquor, withdrawing a portion of said body of liquor rich in potassium compounds from said deposits, reducing the concentration of potassium compounds therein by separating a portion of said potassium compounds, and returning the residual lean liquor to said circulating body.

2. A cyclic process for the solution mining of potassium compounds from underground water soluble deposits containing potassium, magnesium and sulfate ions which comprises circulating a body of aqueous solvent liquor unsaturated with respect to potassium compounds into contact with said deposits, adding a quantity of an inorganic alkaline compound from the group consisting of sodium hydroxide, soda ash, calcium hydroxide, lime and trisodiumphosphate sufficient to raise the pH of said liquor to between 8 and 10 thereby to repress the solubility of the magnesium and sulfate ions in said liquor, withdrawing a portion of said body of liquor rich in potassium compounds from said deposits, reducing the concentration of potassium compounds therein by separating a portion of said potassium compounds and returning the residual lean liquor to said circulating body.

3. A cyclic process for the solution mining of potassium compounds from underground water soluble deposits containing potassium, magnesium and sulfate ions which comprises circulating a body of aqueous solvent liquor unsaturated with respect to potassium compounds into contact with said deposits, adding a quantity of lime sufficient to raise the pH of said liquor to between 8 and 10 thereby to repress the solubility of the magnesium and sulfate ions in said liquor, withdrawing a portion of said body of liquor rich in potassium compounds from said deposits, reducing the concentration of potassium compounds therein by separating a portion of said potassium compounds, and returning the residual lean liquor to said circulating body.

45 References Cited in the file of this patent

UNITED STATES PATENTS

| Number       | Name           | Date          |
|--------------|----------------|---------------|
| 1,466,352    | Dolbear        | Aug. 28, 1923 |
| 50 1,812,497 | Ransom         | June 30, 1931 |
| 1,820,160    | Rusberg        | Aug. 25, 1931 |
| 2,029,623    | Kircher et al. | Feb. 4, 1936  |
| 2,331,890    | Cross          | Oct. 19, 1943 |
| 2,388,009    | Pike           | Oct. 30, 1945 |
| 2,404,550    | Thomsen        | July 23, 1946 |